

(Specimens.)

G. T. CLARE.

MIXED PAINT.

No. 324,230.

Patented Aug. 11, 1885.

Fig 1



Fig. 2



WITNESSES

D. K. Indian  
E. H. Gable

INVENTOR

George Thomas Clare  
per Chas H. Fowler

Attorney

# UNITED STATES PATENT OFFICE.

GEORGE THOMAS CLARE, OF JERSEY CITY, NEW JERSEY.

## MIXED PAINT.

SPECIFICATION forming part of Letters Patent No. 324,230, dated August 11, 1885.

Application filed April 19, 1884. (Specimens.)

*To all whom it may concern:*

Be it known that I, GEORGE THOMAS CLARE, a citizen of the United States, residing at Jersey City, in the county of Hudson and State of New Jersey, have invented certain new and useful Improvements in Printing-Surfaces, both Lithographic and Letter-Press; and I do hereby declare that the following is a full, clear, and exact description of the same, reference being had to the annexed drawings, in which—

Figure 1 is a perspective view in order to illustrate my invention, and Fig. 2 a longitudinal section.

15 My object is to obtain upon the well-known iron, tin, or zinc plates of commerce or any other suitable plate a surface-coating on which designs may be printed by means of ordinary letter-press and lithograph in exactly the same 20 manner as is now produced on card-board.

The following description will give the several ingredients employed in my process, together with the manner of compounding and using the same.

25 I prefer zinc to either iron or tin for flat surfaces, or for surfaces which are required to be only slightly raised or stamped—such, for instance, as clock-dials—tin if to be converted into cans or boxes, iron if for advertising-signs.

30 In order to illustrate my invention, I have shown a suitable sheet, A, provided with the coating B, and printing-surface C, which will be hereinafter described.

35 I mix of tough varnish three parts, raw linseed-oil one part, and add any-colored pigment most likely to assist the next operation. With this I coat the sheet of metal. Up to this point there is nothing special, except that a sheet of zinc, tin, or iron has been coated with a pigment ground in varnish and oil; but it is essential to that which follows. When this varnish and oil coat is passed into a low heat, either in an ordinary japanner's oven or an open warm 40 room, a strong, bright, smooth, and even "tack" is produced, and on this I lay my "picking-up" or printing surface, which is made as follows: If I require a perfectly white enamel-looking surface, suitable, say, for clock-dials, 45 I use as the pigment in the varnish and raw linseed-oil fine French zinc-white, and when

the tack comes I lay one or more coats of the following water-mixtures: best French glue, one pound; water, with one ounce glycerine added, ten pounds; blanc fixe, (in pulp,) two 55 pounds; fine clay, one pound. Soak the glue in half the water; when soft add the other half; heat until dissolved; then add the blanc fixe and clay, and strain. This water-mixture may now be spread on the first or tacky coat by 60 means of a soft brush, and afterward blended down to take out the brush-marks. The result is, first, the varnish and oil coat binds firmly on the metal and raises a tack; second, the water-mixture binds firmly on the tacky 65 coating and will not scale off; third, the water-mixture coating, when dry, leaves a picking-up surface equal to the finest enamel-paper, and may be printed as by the ordinary lithographic or letter-press machines in the ordinary way. The plates may be passed through 70 rollers or not, as may seem necessary; but with ordinary care they will be found to be smooth enough. Any-colored pigment may be used, as the requirements of the work may call for, 75 and gum of any kind soluble in water may be substituted for the glue. I have thus given in detail a full description of the several ingredients used in the compounds employed in my process, together with the manner of using the 80 same, and the relative proportions of such ingredients which I prefer to adopt; but I wish it understood that the proportions may be varied, and therefore I do not confine myself to them precisely as stated.

85 What I claim as new, and desire to secure by Letters Patent, is—

The herein-described composition for forming a printing-surface for metal plates, consisting of glue, water, glycerine, blanc fixe, and 90 clay in substantially the proportions named, and adapted to be applied, as set forth, over a coating of varnish and oil, with a colored pigment, for the purpose specified.

In testimony that I claim the above I have 95 hereunto subscribed my name in the presence of two witnesses.

GEORGE THOMAS CLARE.

Witnesses:

GEORGE H. HOAGLAND,  
WELMER T. JAHNE.